# EUROPEAN PATENT SPECIFICATION

(11) **EP 2 937 427 B1**
(45) Date of publication and mention of the grant of the patent: **05.08.2020**
(21) Application number: 12890530.4
(22) Date of filing: 27.12.2012
(51) Int. Cl.: C21B 13/10, C22B 1/16, C22B 4/08, C22B 5/10, C22B 1/24, C22B 1/245, C22B 19/00, C22B 26/00, C21B 13/00

(54) **REDUCED-IRON PRODUCTION METHOD**
HERSTELLUNGSVERFAHREN FÜR REDUZIERTES EISEN
PROCÉDÉ DE PRODUCTION DE FER RÉDUIT

(30) Priority: 18.12.2012 KR 20120148940
(43) Date of publication of application: 28.10.2015
(73) Proprietor: Posco, Gyeongsangbuk-do 790-300 (KR)
(72) Inventor: SON, Sang Han, Gwangyang-si Jeollanam-do 545-090 (KR); CHO, Byung Kook, Gwangyang-si Jeollanam-do 545-090 (KR); JEONG, Hae Kwon, Gwangyang-si Jeollanam-do 545-090 (KR)
(74) Representative: Zech, Stefan Markus
(86) International application number: PCT/KR2012/011650
(87) International publication number: WO 2014/098300

(56) References cited:
- EP-A1- 2 458 020
- DE-A1- 2 514 325
- JP-A- H09 316 512
- JP-A- H11 131 119
- JP-A- 2010 007 163
- KR-A- 20000 062 353
- KR-B1- 100 516 507
- US-A- 3 443 931

## Description

### Technical Field

The present invention relates to a method for producing reduced iron. More particularly, the present invention relates to a method for producing high reduced rate iron from iron ore abundant in phosphorous, zinc and alkali element impurities, with the concomitant recovery of phosphorous, zinc and alkali elements.

### Background Art

In blast furnaces, convertors or electric furnaces, reduced iron is used as a material for making molten iron or molten steel.

Reduced iron is produced from reduction of an oxidized iron source, such as iron ore or oxidized iron by a carbonaceous reducing agent (hereinafter referred to as "carbonaceous material") or a reducing gas. This process, called direct reduction, is most commonly used to produce reduced iron.

For producing direct reduced iron (DRI), a rotary hearth furnace (RHF) is utilized in which pellets composed of extremely trace iron ore are reduced.

With regard to processes of producing reduced iron using RHF, for example, reference may be made to Korean Patent Application Examined Publication No. 10-2010-0043095 titled "Process for producing reduced iron pellets, and process for producing pig iron"(Patent Document 1), and Korean Patent Application Unexamined Publication No. 10-2010-0122946, titled "Process for production of direct-reduced iron" (Patent Document 2).

Both Patent Documents 1 and 2 are directed to the production of reduced iron using a rotary furnace. In Patent Document 1, particle sizes of raw materials are controlled to improve reactivity, thereby producing a reduced iron pellet in which a metallization ratio is increased while Patent Document 2 discloses the production of iron ore rich in zinc.

Because conventional rotary furnaces are compactly configured to reduce iron ore at up to 1,350°C in a reducing atmosphere, it is difficult to maintain the reducing atmosphere within such furnaces. In addition, conventional rotary furnaces are not suitable for use in mass scale production due to their annual capacity of production amounting only to 150,000 ∼ 500,000 tons.

Due to the limitations of rotary furnaces, a new process is required for the mass production of reduced iron.

In an effort to overcome the limitations of conventional rotary furnaces, production of partially reduced iron under an oxidative atmosphere in a furnace has been suggested. However, the reducing agent carbon is burnt with oxygen from the oxidative atmosphere within the furnace to generate the heat of combustion. That is, since a larger amount of carbon is used as an energy source than as a reducing agent for iron ore, the reduction efficiency of iron ore is poor.

Further, even though iron ore is reduced in a furnace with an oxidative atmosphere, the reduced iron may be re-oxidized by the oxidative atmosphere, which is also a cause of poor reduction rate.

Meanwhile, phosphorus (P), zinc (Zn) and alkali oxides (K₂O+Na₂O) within iron ore are impurities that may cause various defects in the final reduced iron product. Iron ore that has a lower content of phosphorus (P), zinc (Zn), and alkali oxides (K₂O+Na₂O) is preferred.

With the gradual depletion of iron ore having a low impurity content, the cost of quality iron ore has recently increased. Together with the high material cost, the depletion makes it more difficult to produce quality iron ore. In this context, suggestion has been made of a steel making technique characterized by removing the impurities. However, this technique requires various subsidiary materials necessary for the removal of such impurities, and an additional process of removing impurities, thus increasing the production cost. Exemplary methods for producing reduced iron known in the art are described in DE 25 14 325 A1 and EP 2 458 020 A1. JP H09 316512 A discloses an apparatus for producing reduced iron.

### [Related Art Document]

### [Patent Document]

(Patent document 1) Korean Patent Application Unexamined Publication No. 10-2010-0043095 (2010. 04. 27)
(Patent document 2) Korean Patent Application Unexamined Publication No. 10-2010-0122946 (2010. 11. 23)

### Disclosure

### Technical Problem

The present invention provides a method for producing reduced iron under an oxidative atmosphere in an open-type furnace.

In the method and the apparatus, a mixture of iron ore and carbonaceous material is molded into ore agglomerates and sufficiently reduced under an oxidative atmosphere in a reducing furnace.

In addition, the present invention provides a method for producing reduced iron by which a broad spectrum of iron ores including iron ores rich in one or more of phosphorus (P), zinc (Zn), or alkali oxide (K₂O+Na₂O can be used to effectively produce reduced iron.

Also, the present invention provides a method for producing reduced iron by which phosphorus (P), zinc (Zn) and alkali oxides (K₂O+Na₂O) can be separated and recovered from the iron ores.

### Technical Solution

In accordance with an aspect thereof, the present invention provides a method for producing reduced iron, comprising: mixing an iron material bearing phosphorus, zinc and alkali oxides with a carbonaceous material to prepare a mixture, wherein the mixture has a basicity (CaO/SiO₂) of 1 or greater; forming the mixture into ore agglomerates; reducing the ore agglomerates in an open-type reducing furnace, with concomitant removal of phosphorus, zinc and alkali elements from the ore agglomerates; crushing the reduced ore agglomerates to separate reduced iron from phosphorus-bearing slag; and agglomerating the reduced iron while recovering the slag, wherein the carbonaceous material is used in an amount of 10 parts by weight or greater, based on 100 parts by weight of the mixture, wherein the open-type reducing furnace is heated to a temperature of 1,000°C or higher.

In the mixing step, the mixture contains phosphorus (P) in an amount of 0.06 % by weight or greater, zinc (Zn) in an amount of 0.02 % by weight or greater, and an alkali oxide (K₂O+Na₂O) in an amount of 0.1 % by weight or greater.

In one embodiment of the method, the iron material is selected from among an iron ore having a phosphorus (P) content of 0.06 % or greater, an iron ore having a zinc (Zn) content of 0.02 % or greater, an iron ore having an alkali oxide (K₂O+Na₂O) content of 0.1 % or greater, and a combination thereof.

In the mixing step, the carbonaceous material contains carbon-bearing dust generated from a coal mining site or a steelworks or both.

In the mixing step, the mixture has an alkali oxide content of 0.5 % or greater.

In the mixing step, the mixture is further supplemented with a subsidiary material for adjusting basicity and an alkali oxide content, said subsidiary material including CaO to adjust the basicity of the mixture, and Na₂CO₃ and K₂CO₃ to adjust the alkali oxide content of the mixture.

In another embodiment of the present invention, the reducing furnace maintains an oxidative atmosphere therein during the reducing step in which gas is generated upon the reduction of the carbonaceous material within the ore agglomerates, forming a gas film that surrounds the ore agglomerates and thus blocks the ore agglomerates from the oxidative atmosphere.

The open-type reducing furnace is heated to a temperature of 1,000°C or higher to calcine the ore agglomerates, and operated for a limited period of time at maximum such that carbon is completely depleted of the ore agglomerates.

In another embodiment of the present invention, the reducing step comprises recovering the zinc within the ore agglomerates as a dust in an exhaust gas from the open-type furnace, water granulating the recovered dust to separate zinc oxide (ZnO), and recovering the zinc oxide.

In another embodiment of the present invention, wherein the zinc within the ore agglomerates is vaporized during the reduction step in the reducing furnace, discharged together with the exhaust gas, and reacted with oxygen of the exhaust gas to form zinc oxide (ZnO), said zinc oxide being recovered as a dust.

In another embodiment of the present invention, the recovered dust is water granulated during which the alkali element is separated and recovered together with the water.

In another embodiment of the present invention, the reduced iron is separated from the slag using a magnetic seperator.

In accordance with another aspect thereof, the present invention provides a method for producing reduced iron, comprising: mixing an iron material with a carbonaceous material to form ore agglomerates, and reducing the ore agglomerates in an open-type furnace.

In one embodiment of this method, the carbonaceous material is used in an amount of 10 parts by weight or greater, based on 100 parts by weight of the ore agglomerates, and wherein the reducing furnace maintains an oxidative atmosphere therein during the reducing step in which gas is generated upon the reduction of the carbonaceous material within the ore agglomerates, thus forming a gas film that surrounds the ore agglomerates and blocks the ore agglomerates from the oxidative atmosphere.

In accordance with an exemplary embodiment not forming part of the invention, the present application discloses an apparatus of producing reduced iron, comprising: a plurality of raw material hoppers for respectively storing different types of iron ores therein; a carbonaceous material hopper for storing a carbonaceous material therein; a mixer for mixing the effluent of different types of iron ores from the raw material hoppers with the carbonaceous material from the carbonaceous material hopper; a first molding press for forming the mixture into ore agglomerates; an open-type reducing furnace for reducing the ore agglomerates in an oxidative atmosphere; a spaller for crushing the ore agglomerates reduced in the reducing furnace; a magnetic separator for separating the crushed, reduced particles into reduced iron and slag by magnetism; and a second molding press for molding the reduced iron

The apparatus may further comprise: a collector for collecting dust from an exhaust gas from the reducing furnace; and a water granulator for granulating the collected dust with water to separate zinc oxide from alkali element-bearing waste water.

### Advantageous Effects

As described above, iron ores avoided for use in conventional iron making processes due to their high impurity content can be employed for producing reduced iron on a mass scale under an oxidative atmosphere using an open-type furnace in accordance with the present invention.

For a detailed description, the method of the present invention is provided for producing reduced iron, comprising: mixing an iron material with a carbonaceous material to form ore agglomerates; and reducing the ore agglomerates in an open-type furnace, wherein the reducing furnace maintains an oxidative atmosphere therein during the reducing step in which gas is generated upon the reduction of the carbonaceous material within the ore agglomerates, thus forming a gas film that surrounds the ore agglomerates and blocks the ore agglomerates from the oxidative atmosphere.

Further, impurities such as phosphorus (P), zinc (Zn), and alkali oxides (K₂O+Na₂O) contained in iron ores can be utilized in the reducing step, and can be recovered from the iron.

Consequently, a broad spectrum of iron ores can be utilized, which leads to a decrease in the cost of raw materials used in making iron. In addition, phosphorus (P), zinc (Zn) and alkali oxides (K₂O+Na₂O) can be recovered the process.

### Description of Drawings

FIG. 1 is a schematic view illustrating an apparatus of and a method for producing reduced iron.
FIG. 2 is a graph illustrating phosphorus recovery rates in slag versus basicity after the reduction of ore agglomerates at 1,200ºC for 20 min.
FIG. 3 is a graph illustrating phosphorus recovery rates of slag versus alkali oxide content in ore agglomerates after the reduction of ore agglomerates having a basicity of 1 at 1200ºc for 20 min.
FIG. 4 is a graph showing the metallization ratio of ore agglomerates versus the temperature of the open-type reducing furnace according to the amount of the carbonaceous material.

### Best Mode

Embodiments of the present invention are described with reference to the accompanying drawings in order to describe the present invention in detail so that those having ordinary knowledge in the technical field to which the present invention pertains can easily practice the present invention. It should be noted that same reference numerals are used to designate the same or similar elements throughout the drawings. In the following description of the present invention, detailed descriptions of known functions and configurations which are deemed to make the gist of the present invention obscure will be omitted.

First, a description will be given of an apparatus by which a method for producing reduced iron can be embodied in accordance with an embodiment of the present ivnention.

With reference to FIG. 1, there is a schematic view illustrating an apparatus and method for producing reduced iron.

As can be seen FIG. 1, the apparatus of producing reduced iron comprises a first spaller 11 for crushing iron ore; a plurality of hoppers 21, 22 and 23 for storing the iron ore crushed in the first spaller 11 by type therein; a second spaller 12 for crushing a carbonaceous material, such as coal; a carbonaceous material hopper 30 for storing the carbonaceous material crushed by the second spaller 12 therein; a mixer 50 for mixing effluent from different types of iron ore from the raw material hoppers 21, 22 and 23 with the crushed carbonaceous material from the carbonaceous material hopper 30; a first molding press 61 for forming the mixture into ore agglomerates; an open-type reducing furnace 70 for reducing the ore agglomerates in an oxidative atmosphere; a third spaller 13 for crushing the ore agglomerates reduced in the reducing furnace 70; a magnetic separator 80 for separating the crushed, reduced particles into reduced iron and slag by magnetism; and a second molding press 62 for molding the reduced iron. Optionally, the apparatus may further comprise at least one subsidiary material hopper 40 for storing a subsidiary material therein; a collector 90 for collecting dust from an exhaust gas from the reducing furnace; and a water granulator 100 for granulating the collected dust with water to separate zinc oxide from alkali element-bearing waste water.

The open-type reducing furnace has an internal space that is open rather than closed. So long as it can heat ore agglomerates while continuously transporting the ore agglomerates, any reducing furnace, without limitations to specific configurations, may be employed. By way of example, an open-type reducing furnace may be provided with a transport means for transporting ore agglomerates in a conveyer manner. A furnace body defining an internal space in which the ore agglomerates are conveyed and reduced is located above the transport means. The internal space of the furnace body is heated by a plurality of burners installed therein. In addition, a suction means for aspirating air from the internal space of the furnace body is provided below the transport means. In this structure, ore agglomerates are conveyed by the transport means while heat flows downwardly from an upper space of the ore agglomerates by the combustion of the burners and the aspiration of the suction means. In such an open-type furnace, ore agglomerates can be arranged in a multi-layer pattern and can be continuously reduced to produce reduced iron on a mass scale.

Each of the first molding press 61 and the second molding press 62 is a twin role structure.

Next, the production of reduced iron using the apparatus illustrated above will be described.

Various iron ores are crushed in the first spaller 11 shown in FIG. 1 and individually stored in the iron raw hoppers 21, 22 and 23 by type. The iron ores may have a phosphorus (P) content of 0.06 % or greater, a zinc (Zn) content of 0.02 % or greater, an alkali oxide (K₂O+Na₂O) content of 0.1 % or greater, or a combination thereof. Separately, a carbonaceous material is crushed in the second spaller 12 and stored in the carbonaceous material hopper 30. The carbonaceous material may contain carbon-bearing dust generated from a coal mining site or a steelworks or both. In this regard, the carbonaceous material preferably has a particle size of 0.1 mm or less so as to enhance reactivity.

In addition, the subsidiary material hopper 40 stores a subsidiary material for adjusting basicity and a subsidiary material for adjusting the content of alkali oxides, in combination or separately, therein. For instance, CaO may be used as a subsidiary material for adjusting basicity, and the content of alkali oxides may be adjusted with Na₂CO₃ or K₂CO₃ or both.

After being prepared like this, the iron ore, the carbonaceous material, and the subsidiary materials are each weighed, introduced into the mixer 50, and mixed to give a mixture.

Preferably, the mixture comprises phosphorus (P) in an amount of 0.06 % or greater, zinc (Zn) in an amount of 0.02 % or greater, and an alkali oxide (K₂O+Na₂O) in an amount of 0.1 % or greater, which are mostly derived from the iron ore and the carbonaceous material. However, the ore agglomerates, as will be described later, are preferably maintained to have a high basicity and a high alkali oxide content in order to sufficiently isolate phosphorus during the reduction of ore agglomerates. Accordingly, CaO, Na₂CO₃, and K₂CO₃ are preferably added in such amounts as to adjust the basisicity (CaO/SiO₂) of the mixture to 1 or higher and to maintain an alkali oxide content of 0.5 % in the mixture. The reason why the basicity and the alkali oxide content are limited will be revealed later in the description given in conjunction with FIGS. 2 and 3.

The mixture thus obtained is fed to the first molding press 61 where homogeneously sized ore agglomerates are formed.

Subsequently, the ore agglomerates are introduced into the open-type reducing furnace 70 where iron (Fe) of the ore agglomerates is reduced in an oxidative atmosphere while separating phosphorus, zinc and alkali elements from the iron. In this context, the oxidative atmosphere means exposure to air without any atmospheric control.

Reactions in the reduction process will be detailed. Iron oxides within the ore agglomerates react (are reduced), as shown in the following Chemical Formula 1, to generate Fe and CO. Then, this CO reacts with (reduces) the iron oxides of the ore agglomerates as shown in the following Chemical Formula 2, with the concomitant generation of iron (Fe) and CO₂. This CO₂ may be converted into CO by reaction with carbon within the ore agglomerates. The CO and CO₂ gases that are generated by reactions between iron oxides and carbon within the ore agglomerates are exhausted externally, forming a gas film surrounding the ore agglomerates. As the gas film serves to block the ore agglomerates from the oxidative atmosphere of the open-type reducing furnace 70, the reduction of the ore agglomerates can be facilitated in the open-type reducing furnace 70.

According to the invention, a sufficient amount of the gas film is formed by fully reacting iron oxides of the ore agglomerates with carbon. For this, a sufficient amount of carbon is contained in the ore agglomerates. In this regard, the carbonaceous material is mixed in an amount of 10 parts by weight or greater, based on 100 parts by weight of the total mixture.

In addition, the open-type reducing furnace 70 is maintained to have a calcination temperature of 1,000ºC or higher to reduce the ore agglomerates.

FIG. 4 is a graph showing the metallization ratio of ore agglomerates versus the temperature of the open-type reducing furnace according to the amount of the carbonaceous material. As can be seen, ore agglomerates containing a carbonaceous material in an amount of 10 parts by weight were found to allow sufficient metallization.

Since the gas film is formed as a result of a reaction with the carbon of the ore agglomerates, the time of the reduction of the ore agglomerates is preferably limited at maximum to an extent that carbon is completely depleted of the ore agglomerates.

During the reduction of the ore agglomerates in the open-type furnace 70, phosphorus, oxygen and CaO elements of the ore agglomerates undergo a reaction to form a slag containing the elements in the form of, for example, CaO·(P₂O₅). Hence, the ore agglomerates are in the mixture of reduced iron and slag.

Turning to zinc contained in the ore agglomerates, zinc oxide and alkali oxides (K₂O+Na₂O) are reduced at lower temperatures than are iron oxides, and are discharged as an exhaust gas.

When discharged together with the exhaust gas, the zinc (Zn) vaporized during the reduction of the ore agglomerates reacts with oxygen in the exhaust gas to form a zinc oxide (ZnO) that is then collected as a dust by the collector 90.

During the reduction of the ore agglomerates, the alkali elements are also vaporized, exhausted as a gas, and reacted with oxygen of the exhaust gas to form an alkali oxide. Likewise, this oxide is collected as a dust by the collector 90.

After the dust collected by the collector 90 is treated in the water granulator 100, waste water containing crude zinc oxide and alkali elements is recovered.

Meanwhile, the ore agglomerates in mixture with reduced iron and slag are crushed in the third spaller 13 and separated into reduced iron and slag by magnetism in the magnetic separator 80. The reduced iron thus obtained is formed into briquettes of a predetermined size in the second molding press 62 while the slag rich in CaO and phosphorus may be recycled as a fertilizer material.

### EXAMPLES

A better understanding of the present invention may be obtained through the following examples that are set forth to illustrate, but are not to be construed as limiting the present invention.

Compositions of iron ores used in experiments are summarized in Table 1, below.

Iron ores rich in phosphorus, zinc and alkali elements (Na₂O, K₂O) were used. Each iron ore was formed into briquettes rich in phosphorus, zinc and alkali elements. Optionally, zinc oxide, phosphorus oxide and alkali oxides, all in a reagent grade, were added to maximize contents of zinc, phosphorus and alkali elements.

For comparison, the composition of an iron ore that is used in a typical iron making process (iron ore C) is also given in Table 1. As can be in Table 1, iron ore C, which is used in a typical iron making process, has a phosphorus content of about 0.06% or less, a zinc content of about 0.02 % or less, and an alkali oxide content of 0.03 % or less whereas both iron ores A and B are relatively rich in phosphorus, zinc, and alkali oxide.

**TABLE 1**

| Classification | T. Fe | SiO₂ | Al₂O₃ | CaO | MgO | P | Zn | K₂O | Na₂O |
|---|---|---|---|---|---|---|---|---|---|
| Iron Ore A | 41.1 | 17.8 | 2.41 | 3.20 | 13.7 | 0.013 | 0.103 | 0.687 | - |
| Iron Ore B | 55.3 | 8.5 | 0.90 | 4.38 | 0.21 | 0.52 | 0.019 | 0.039 | 0.10 |
| Iron Ore C | 65.7 | 1.87 | 1.19 | 0.01 | 0.09 | 0.023 | 0.009 | 0.036 | 0.012 |

Iron ores A and B were independently mixed with coal (20 % by weight) and formed into briquettes. In order to increase basicity and alkali oxide content in the briquettes, CaO, K₂O, and Na₂O in a reagent grade were added. Under a reducing furnace simulated condition, the briquettes were reduced.

A reduction experiment was carried out on the briquettes by elevating the temperature at a rate of 50ºC/min to a reduction temperature of 1,200ºC and by maintaining the reduction temperature for 20 min. Then, the briquettes were analyzed for Fe, Zn, and P content while Fe, Zn, P, K, and Na content in the slag is examined.

FIG. 2 is a graph illustrating phosphorus recovery rates in slag versus basicity after the reduction of ore agglomerates at 1,200ºC for 20 min, and FIG. 3 is a graph illustrating phosphorus recovery rates of slag versus alkali oxide content in ore agglomerates after the reduction of ore agglomerates having a basicity of 1 at 1200ºC for 20 min.

As is understood from data of FIG. 2, the phosphorous recovery rate in slag gradually increases with an increase in basicity. As for the phosphorus oxide (P₂O₅), its stability is maintained in the condition of high basicity. Particularly, phosphorus oxide in the slag is stable even when a strong alkali such as alkali oxide is added. Therefore, the addition of small amounts of highly basic slag and alkali oxide is effective in preventing phosphorus oxide from being reduced and dissolved into the metal Fe during the reduction of reduced iron, and thus in allowing phosphorus oxide to exist in the slag.

After completion of the experiment, the briquettes were found to have a reduction rate of approximately 85 ∼ 90% irrespective of basicity. In addition, the zinc content in the slag after reduction was decreased to approximately 0.004 % from 0.1 % in the initial phase. Reduction of zinc oxide to metal Zn occurred at a lower temperature than reduction of iron oxide to its metal. Soon after reduction into metal zinc, it was vaporized, exhibiting a high vapor pressure. The gaseous zinc was re-oxidized into and discharged as ZnO in exhaust gas.

As can be seen in FIG. 3, the recovery rate of phosphorous in slag was observed to increase with an increase in the alkali oxide content of the briquettes. Hence, the use of alkali oxide-rich iron ore in mixture with phosphorus-rich iron ore is advantageous in enhancing phosphorus recovery rates in slag. Accordingly, it was found that phosphorus could be recovered to a desired degree when the mixture was set to have a basicity (CaO/SiO₂) of 1 or higher, and an alkali oxide content of 0.5 % or higher.

Although the preferred embodiments of the present invention have been disclosed for illustrative purposes, those skilled in the art will appreciate that various modifications, additions and substitutions are possible, without departing from the scope of the accompanying claims.

### <Description of the Reference Numerals in the Drawings>

- 11, 12, 13:: Spaller,
- 21, 22, 23:: raw material hopper
- 30:: carbonaceous material hopper
- 40:: subsidiary material hopper
- 50:: mixer
- 61,: 62: molding press
- 70:: open-type reducing furnace
- 80:: magnetic separator
- 90:: collector
- 100:: water granulator

## Claims

1. A method for producing reduced iron, comprising:
mixing an iron material bearing phosphorus, zinc and alkali oxides with a carbonaceous material to prepare a mixture, wherein the mixture has a basicity (CaO/SiO₂) of 1 or greater;
forming the mixture into ore agglomerates;
reducing the ore agglomerates in an open-type reducing furnace, with concomitant removal of phosphorus, zinc and alkali elements from the ore agglomerates;
crushing the reduced ore agglomerates to separate reduced iron from phosphorus-bearing slag; and
agglomerating the reduced iron while recovering the slag, wherein the carbonaceous material is used in an amount of 10 parts by weight or greater, based on 100 parts by weight of the mixture,
wherein the open-type reducing furnace is heated to a temperature of 1,000°C or higher.

2. The method of claim 1, wherein the mixture contains phosphorus (P) in an amount of 0.06 % by weight or greater, zinc (Zn) in an amount of 0.02 % by weight or greater, and an alkali oxide (K₂O+Na₂O) in an amount of 0.1 % by weight or greater.

3. The method of claim 2, wherein the iron material is selected from among an iron ore having a phosphorus (P) content of 0.06 % or greater, an iron ore having a zinc (Zn) content of 0.02 % or greater, an iron ore having an alkali oxide (K₂O+Na₂O) content of 0.1 % or greater, and a combination thereof.

4. The method of claim 1, wherein the carbonaceous material contains carbon-bearing dust generated from a coal mining site or a steelworks or both.

5. The method of claim 1, wherein the mixture has an alkali oxide content of 0.5 % or greater.

6. The method of claim 1 or 5, wherein the mixture is further supplemented with a subsidiary material for adjusting basicity and an alkali oxide content, said subsidiary material including CaO to adjust the basicity of the mixture, and Na₂CO₃ and K₂CO₃ to adjust the alkali oxide content of the mixture.

7. The method of claim 1, wherein the reducing furnace maintains an oxidative atmosphere therein during the reducing step in which gas is generated upon the reduction of the carbonaceous material within the ore agglomerates, forming a gas film that surrounds the ore agglomerates and thus blocks the ore agglomerates from the oxidative atmosphere.

8. The method of claim 1, wherein the reducing step comprises recovering the zinc within the ore agglomerates as a dust in an exhaust gas from the open-type furnace and water granulating the recovered dust to separate zinc oxide (ZnO), and recovering the zinc oxide.

9. The method of claim 8, wherein the zinc within the ore agglomerates is vaporized during the reduction step in the reducing furnace, discharged together with the exhaust gas, and reacted with oxygen of the exhaust gas to form zinc oxide (ZnO), said zinc oxide being recovered as a dust.

10. The method of claim 8, wherein the recovered dust is water granulated during which the alkali element is separated and recovered together with water.

11. The method of claim 1, wherein the reduced iron is separated from the slag using a magnetic separator.

## Patentansprüche

1. Verfahren zur Herstellung von reduziertem Eisen, umfassend:
Mischen eines Eisenmaterials, das Phosphor, Zink und Alkalioxide enthält, mit einem kohlenstoffhaltigen Material, um ein Gemisch herzustellen,
wobei das Gemisch eine Basizität (CaO/SiO₂) von 1 oder mehr aufweist;
Formen des Gemisches zu Erzagglomeraten;
Reduzieren der Erzagglomerate in einem Reduktionsofen vom offenen Typ mit gleichzeitiger Entfernung von Phosphor, Zink und Alkalielementen aus den Erzagglomeraten;
Brechen der reduzierten Erzagglomerate, um reduziertes Eisen von phosphorhaltiger Schlacke abzuscheiden; und
Agglomerieren des reduzierten Eisens, während die Schlacke rückgewonnen wird, wobei das kohlenstoffhaltige Material in einer Menge von 10 Gewichtsteilen oder mehr basierend auf 100 Gewichtsteilen des Gemisches verwendet wird,
wobei der Reduktionsofen vom offenen Typ auf eine Temperatur von 1.000 °C oder mehr erhitzt wird.

2. Verfahren nach Anspruch 1, wobei das Gemisch Phosphor (P) in einer Menge von 0,06 Gew.-% oder mehr, Zink (Zn) in einer Menge von 0,02 Gew.-% oder mehr und ein Alkalioxid (K₂O + Na₂O) in einer Menge von 0,1 Gew.-% oder mehr enthält.

3. Verfahren nach Anspruch 2, wobei das Eisenmaterial aus einem Eisenerz mit einem Gehalt an Phosphor (P) von 0,06 % oder mehr, einem Eisenerz mit einem Gehalt an Zink (Zn) von 0,02 % oder mehr, einem Eisenerz mit einem Gehalt an Alkalioxid (K₂O + Na₂O) von 0,1 % oder mehr und einer Kombination davon ausgewählt wird.

4. Verfahren nach Anspruch 1, wobei das kohlenstoffhaltige Material Kohlenstoff enthaltenden Staub enthält, der aus einem Kohlebergwerk oder einem Stahlwerk oder beidem gewonnen wird.

5. Verfahren nach Anspruch 1, wobei das Gemisch einen Alkalioxid-Gehalt von 0,5 % oder mehr aufweist.

6. Verfahren nach Anspruch 1 oder 5, wobei das Gemisch ferner mit einem Zusatzmaterial zum Einstellen der Basizität und eines Alkalioxid-Gehalts ergänzt wird, wobei das Zusatzmaterial CaO zum Einstellen der Basizität des Gemisches und Na₂CO₃ und K₂CO₃ zum Einstellen des Alkalioxid-Gehalts des Gemisches beinhaltet.

7. Verfahren nach Anspruch 1, wobei der Reduktionsofen während des Reduktionsschritts eine oxidierende Atmosphäre in ihm aufrechterhält, wobei Gas bei der Reduktion des kohlenstoffhaltigen Materials in den Erzagglomeraten erzeugt wird, wodurch ein Gasfilm gebildet wird, der die Erzagglomerate umgibt und so die Erzagglomerate gegenüber der oxidierenden Atmosphäre abblockt.

8. Verfahren nach Anspruch 1, wobei der Reduktionsschritt das Rückgewinnen des Zinks in den Erzagglomeraten als Staub in einem Abgas aus dem Ofen vom offenen Typ und das Wassergranulieren des rückgewonnenen Staubs zur Abscheidung von Zinkoxid (ZnO) und das Rückgewinnen des Zinkoxids umfasst.

9. Verfahren nach Anspruch 8, wobei das Zink in den Erzagglomeraten während des Reduktionsschritts im Reduktionsofen verdampft wird, zusammen mit dem Abgas abgeführt wird und mit Sauerstoff des Abgases umgesetzt wird, um Zinkoxid (ZnO) zu bilden, wobei das Zinkoxid als Staub rückgewonnen wird.

10. Verfahren nach Anspruch 8, wobei der rückgewonnene Staub wassergranuliert wird, wobei das Alkalielement dabei abgeschieden wird und zusammen mit Wasser rückgewonnen wird.

11. Verfahren nach Anspruch 1, wobei das reduzierte Eisen mithilfe eines Magnetabscheiders von der Schlacke abgeschieden wird.

## Revendications

1. Procédé de production de fer réduit, comprenant :
le mélange d'un matériau de fer porteur de phosphore, de zinc et d'oxydes alcalins avec un matériau carboné pour préparer un mélange, dans lequel le mélange a une basicité (CaO/SiO₂) de 1 ou plus ;
la formation du mélange en agglomérats de minerai ;
la réduction des agglomérats de minerai dans un four de réduction de type ouvert, avec l'élimination concomitante de phosphore, de zinc et d'éléments alcalins des agglomérats de minerai ;
le broyage des agglomérats de minerai réduits pour séparer du fer réduit de scories porteuses de phosphore ; et
l'agglomération du fer réduit tout en récupérant les scories, dans lequel le matériau carboné est utilisé dans une quantité de 10 parties en poids ou plus, pour 100 parties en poids du mélange,
dans lequel le four de réduction de type ouvert est chauffé à une température de 1 000 °C ou plus.

2. Procédé selon la revendication 1, dans lequel le mélange contient du phosphore (P) dans une quantité de 0,06 % en poids ou plus, du zinc (Zn) dans une quantité de 0,02 % en poids ou plus, et un oxyde alcalin (K₂O + Na₂O) dans une quantité de 0,1 % en poids ou plus.

3. Procédé selon la revendication 2, dans lequel le matériau de fer est choisi parmi un minerai de fer ayant une teneur en phosphore (P) de 0,06 % ou plus, un minerai de fer ayant une teneur en zinc (Zn) de 0,02 % ou plus, un minerai de fer ayant une teneur en oxyde alcalin (K₂O + Na₂O) de 0,1 % ou plus, et une combinaison de ceux-ci.

4. Procédé selon la revendication 1, dans lequel le matériau carboné contient une poussière porteuse de carbone générée à partir d'un site d'exploitation de charbon ou d'une aciérie ou des deux.

5. Procédé selon la revendication 1, dans lequel le mélange a une teneur en oxyde alcalin de 0,5 % ou plus.

6. Procédé selon la revendication 1 ou 5, dans lequel le mélange est en outre complété avec un matériau subsidiaire pour ajuster la basicité et une teneur en oxyde alcalin, ledit matériau subsidiaire comportant du CaO pour ajuster la basicité du mélange, et du Na₂CO₃ et du K₂CO₃ pour ajuster la teneur en oxyde alcalin du mélange.

7. Procédé selon la revendication 1, dans lequel le four de réduction maintient une atmosphère oxydative en son sein pendant l'étape de réduction dans laquelle du gaz est généré lors de la réduction du matériau carboné au sein des agglomérats de minerai, formant un film de gaz qui entoure les agglomérats de minerai et bloque ainsi les agglomérats de minerai vis-à-vis de l'atmosphère oxydative.

8. Procédé selon la revendication 1, dans lequel l'étape de réduction comprend la récupération du zinc au sein des agglomérats de minerai sous forme de poussière dans un gaz d'échappement provenant du four de type ouvert et la granulation à l'eau de la poussière récupérée pour séparer de l'oxyde de zinc (ZnO), et la récupération de l'oxyde de zinc.

9. Procédé selon la revendication 8, dans lequel le zinc au sein des agglomérats de minerai est vaporisé pendant l'étape de réduction dans le four de réduction, évacué conjointement avec le gaz d'échappement, et mis à réagir avec de l'oxygène du gaz d'échappement pour former de l'oxyde de zinc (ZnO), ledit oxyde de zinc étant récupéré sous forme de poussière.

10. Procédé selon la revendication 8, dans lequel la poussière récupérée est granulée à l'eau, pendant cela, l'élément alcalin est séparé et récupéré conjointement avec l'eau.

11. Procédé selon la revendication 1, dans lequel le fer réduit est séparé des scories à l'aide d'un séparateur magnétique.
